

Feb. 23, 1965

J. G. LANNING

3,170,504

CERAMIC BURNER PLATE

Filed June 5, 1962

3 Sheets-Sheet 1

Fig. 1



Fig. 2.



INVENTOR.  
JOHN G. LANNING  
BY  
Clarence R. Petty, Jr.  
ATTORNEY

Feb. 23, 1965

J. G. LANNING

3,170,504

CERAMIC BURNER PLATE

Filed June 5, 1962

3 Sheets-Sheet 2



INVENTOR.  
John G. Lanning

BY  
Clarence R. Petty  
ATTORNEY

Feb. 23, 1965

J. G. LANNING  
CERAMIC BURNER PLATE

3,170,504

Filed June 5, 1962

3 Sheets-Sheet 3

Fig. 7



INVENTOR.  
JOHN G. LANNING  
BY  
Clarence R. Petty, Jr.  
ATTORNEY

1

3,170,504

**CERAMIC BURNER PLATE**

John G. Lanning, Corning, N.Y., assignor to Corning Glass Works, Corning, N.Y., a corporation of New York

Filed June 5, 1962, Ser. No. 200,235  
8 Claims. (Cl. 158—116)

This invention relates to ceramic burner plates for infrared radiating gas burners and the like. In particular, it comprises a burner plate having an improved and novel combustion surface configuration or geometry.

Heretofore, ceramic burner plates have been constructed in the form of a perforated or honeycomb structure having a plurality of small unobstructed gas passages or open-ended cells separated from each other by thin ceramic walls. The gas passages extend through the burner plate from one major face of the plate to an opposed or opposite major face thereof. One of these major faces constitutes an external combustion surface when the plate is placed over an opening in a gas burner mixing chamber in such a manner that the other major face confronts the interior of the mixing chamber. The combustion surface of these plates is made with a flat, generally smooth configuration to provide an infrared radiating surface as the gaseous fuel burns on the combustion surface after passing through the gas passages from the mixing chamber. Typical examples of this type of ceramic burner plate are those disclosed in United States patent application Serial No. 189,785, filed April 24, 1962, by C. L. Goss and L. C. Liptak, assigned to the assignee of the present application, and in United States Patent No. 2,775,294 to G. Schwank.

It has been found that the flat combustion surface of these burner plates is not uniformly heated by the burning fuel because of slight differences in the thickness of the cell walls and hydraulic diameters of the cells, which is an inherent result of the methods of manufacturing these plates. These differences create sufficient combustion variation to cause uneven heating and, as a result, the flat surface has a mottled appearance. This mottled surface appearance varies considerably in temperature from the orange-white high temperature areas to the dull red or grey low temperature areas. Such a surface condition is undesirable since the maximum conversion of the available B.t.u. content of the gas into infrared energy is not being achieved.

It is an object of this invention to provide a ceramic burner plate having a novel combustion surface configuration or geometry whereby the thermal gradients or uneven heating of the radiating combustion surface due to slight differences in the thickness of the cell walls and hydraulic diameters of the cells is eliminated or greatly reduced.

It is another object of this invention to provide a ceramic burner plate having a novel combustion surface configuration or geometry whereby much more efficient combustion is effected by the resulting thermocatalytic combustion.

It is a further object of this invention to provide a ceramic burner plate having a novel combustion surface configuration or geometry which affords a maximum realization of the available heat content of the gaseous fuel and thereby results in increased temperature of the radiating combustion surface and in greater burner efficiency.

It is a still further object of this invention to provide a ceramic burner plate having a novel combustion surface configuration or geometry that affords an increase in the effective infrared radiating surface area without increasing the overall size of the burner plate, which results in a more efficient combustion of the gaseous fuel and in

2

a more uniform infrared heat radiation over the entire combustion surface.

These and other objects, which will become apparent to those skilled in the art from the detailed description given hereinafter and from the accompanying drawings, are attained in accordance with my discoveries by providing a ceramic gas burner plate comprising a thin wall ceramic, perforated or honeycomb structure having two opposed major faces with a plurality of small gas flow passages extending between the opposed major faces and with one major face comprising a plurality of substantially uniform or purposely irregular peaked protrusions, which may be generally of pyramidal or conical shape, disposed substantially uniformly or purposely irregularly over substantially the entire area or a given portion of this one major face. As a general rule, it is preferred to provide the peaked protrusions with substantially pointed tips, apexes or vertices; however, such apexes may be somewhat rounded, blunted or irregular if desired. Also, by "a plurality of peaked protrusions," it is meant that adjacent peaked protrusions form valleys therebetween by the intersecting or meeting of the downwardly sloping surfaces of the adjacent peaked protrusions. Preferably, the lowermost portion of these valleys are substantially V-shaped, although, if desired, these lowermost portions can be somewhat rounded or flattened in nature.

In the drawings:

FIGURE 1 is a sectional oblique view of an infrared gas burner with one embodiment of a burner plate of the invention;

FIGURE 2 is a sectional view of an infrared gas burner like that shown in FIGURE 1 taken along line II-II;

FIGURE 3 is a sectional isometric view of another embodiment of a burner plate of the invention;

FIGURE 4 is a fragmentary side sectional view of a burner plate of the invention;

FIGURE 5 is a fragmentary side sectional view of a burner plate of the type prior to this invention;

FIGURE 6 is an enlarged fragmentary sectional view of the burner plate structure shown in FIGURE 2; and

FIGURE 7 is graph showing combustion surface temperature as a function of the included angle  $\theta$  shown in FIGURE 4.

Referring now to the drawings, FIGS. 1 and 2 show a gas burner composed of a body member 10 having side walls 12 and a bottom wall 14. Attached to body member 10 is a centrally disposed inlet tube 16 extending from one side wall 12. The top surface or cover plate 18 of the gas burner is a ceramic honeycomb structure comprising one embodiment of a burner plate according to the present invention. The zone 20 within the body 10 between the burner plate 18 and the bottom wall 14 comprises a mixing chamber where air and the fuel, such as natural gas, propane, butane, manufactured gas, town gas or the like, thoroughly mix after entering from inlet tube 16 and prior to passing upwardly through the cover plate 18 for combustion on the upper surface thereof.

The honeycomb burner plate 18 is fitted and attached to the body 10 at the upper portion of the side walls 12 by any suitable means, such as cement or packing 22.

As is shown in the drawings, the honeycomb burner plate 18 is characterized by a large number of unobstructed gas paths or open-ended cells 25 that extend from the bottom or inlet surface 27 of the burner plate through to its top or combustion surface 28. These unobstructed gas paths are defined and separated from one another by thin ceramic walls 30. By unobstructed, I mean that no structure exists within the gas flow paths that would prevent flow. The ceramic walls defining those flow paths can be arranged in triangular, circular or polygonal shape as desired.

The major characterizing feature of the invention is the geometry or configuration of the combustion surface 28, which comprises a plurality of substantially uniform or purposely irregular peaked protrusions disposed substantially uniformly or purposely irregular over substantially the entire area of, or a given portion of, surface 28, as shown in FIGURES 1 and 4. These peaked protrusions are shown to be pyramidal shape in FIGURE 1, but they can also be conically shaped, if desired, as shown in FIGURE 3. In this latter embodiment, the honeycomb burner plate 31 is characterized by a large number of unobstructed gas paths 25 defined and separated from one another by thin ceramic walls 34. These gas paths extend from the bottom or inlet surface 32 through to the top or combustion surface 33.

In the use of a burner plate of the invention, a source of a gaseous fuel and air enter the burner body 10 through the inlet tube 12 or any other suitable inlet means. The fuel and air can be provided by sources connected to a mixing head that is attached to the inlet means, or the pressure of the fuel gas can be used with suitable means to aspirate air into the stream.

Other procedures, none of which form any part of the invention, can be used as well. The gases enter the enlarged space 20 within the burner body 10 and thoroughly mix therein. For mixing purposes, the inlet tube can be designed so that the gases impinge on a wall of the body member 10, or baffles (not shown) can be included within the body or tube to effect that object. The mixed gases then pass through the gas paths 25 in the burner plate 30 to the upper surface 28 where they are combusted, heating the surface of the plate to nearly incandescence. Any suitable conventional combustion initiator can be used as desired.

The significant improvements afforded by the burner plate of the invention are believed to be due to interparticle reinforcement. Thus, as shown in FIGURE 4, a surface particle 35 in the heated surface 28 radiates heat energy in a hemispherical pattern as indicated at 37. With a burner plate according to this invention, having a combustion surface comprising a multitude of peaked protrusions, it can be seen that a substantial amount of the hemispherical radiation of each surface particle will impinge on other surface particles on adjacent peaked protrusions. This effect, which I call interparticle reinforcement, results in increasing the overall temperature of the combustion or radiating surface 28 for any given volume of gaseous fuel per unit of time. In turn, this higher surface temperature promotes thermocatalytic combustion and more complete combustion of the gaseous fuel thereby liberating maximum heat content from the fuel to further increase the combustion surface temperature. As will be apparent, the higher surface temperatures, provided by the burner plate of the invention, increase the amount of radiant energy relative to convected energy for any given unit volume of gaseous fuel combusted; thus the invention affords a significantly greater infrared burner efficiency. Moreover, the geometry or configuration of the peaked protrusions provide a substantially increased area for radiation of infrared energy from the combustion surface thereby producing a more uniform and wider dispersion of infrared heat emission from the combustion surface of the burner plate.

The significance of the improved burner plate of the invention can best be seen by comparing FIGURES 4 and 5. FIGURE 5 shows a burner plate of the type made prior to this invention having a flat combustion surface 40. A surface particle 41 radiates energy in the hemispherical pattern as shown at 42. As can be seen, substantially none of the hemispherical radiation impinges on other surface particles. Thus, interparticle reinforcement is substantially wholly absent.

As was mentioned earlier, a particularly undesirable problem was the development of thermal gradients on the

radiating combustion surface due to the slight differences in the thickness of the cell walls and hydraulic diameters of the cells. This problem can best be understood by reference to FIGURE 6. The honeycomb structure is made of thin ceramic sheets 30 sintered together as at points 45 to form the thin walls defining the gas paths 25. The wall thickness at points 45 are essentially double that of the remaining wall portions. It is at these points that "dark" or cool zones are seen on the edges of the thin ceramic walls making up a flat combustion surface. However, with a peaked combustion surface burner plate of this invention, the hemispherical reinforcement radiation from adjacent peaked protrusions causes these thicker wall edge points 45 to heat up more uniformly with all other areas on the combustion surface. It can also be seen in FIG. 6 that if the cross-sectional areas of the gas passages vary one from another (e.g. if the cross-sectional area of passage 25a is somewhat larger than that of passage 25b), the hydraulic radius then varies and the gas mixture velocity through these passages also varies since the pressure drop from the inlet end of the passages to the outlet end of the passages is the same for each passage. This variation in the velocity of the gas/air mixture causes an uneven burning condition at the combustion surface. This results in uneven surface temperatures and the characteristic mottled appearance of the combustion surface. However, with a peaked combustion surface burner plate, this tendency toward uneven surface temperatures, due to slight variations in the hydraulic diameter of the gas/air mixture flow passages, is substantially reduced. This is substantially a result of the interparticle reinforcement described above.

The areas where the hydraulic diameter is less than the normal (and on a flat combustion surface results in the darker color and lower temperature) interparticle reinforcement due to a peaked combustion surface raises the temperature. This results because the total radiation from the hotter areas is greater than that from the cooler areas as taught by the Stefan-Boltzmann law. Thus, since in a peaked combustion surface, the cooler areas are "seen" by the hotter areas, the cooler areas receive radiation energy from the hotter areas and the temperature differential between the two areas is substantially reduced.

The combustion surface configuration of burner plates according to this invention should have certain particular characteristics that are necessary for practical results. One important characteristic is an appropriate included angle  $\theta$  (see FIGURE 4) relationship between adjacent pyramidal or conical surfaces. The angle  $\theta$  should be between about  $20^\circ$  and  $120^\circ$ , and preferably between  $30^\circ$  and  $90^\circ$ . The significance of this angular relationship can best be seen by reference to FIGURE 7 wherein combustion surface temperature data is shown as a function of the included angle  $\theta$ . The data was obtained by solely varying the angle  $\theta$  and maintaining all other factors (e.g. burner plate dimensions, fuel, etc.) the same. The temperature measurements were made by focusing a radiant energy detecting pyrometer 45 (see FIGURE 4) on the combustion surface at an angle  $\alpha$  of  $30^\circ$  to the normal of the general plane of that surface. The plot of data for an angle  $\alpha$  of  $30^\circ$  to the normal is shown in FIGURE 7 as merely one convenient illustration of the pattern of variation in combustion surface temperature with variation of the included angle  $\theta$ . Similar patterns of variation between combustion surface temperature and included angle  $\theta$  are found with an angle  $\alpha$  of  $0^\circ$  to  $60^\circ$ . Thus, as shown in FIGURE 7, angles of greater than about  $120^\circ$  do not produce enough interparticle reinforcement for practical results of increased combustion surface temperature and of maximizing combustion of the gaseous fuel. Angles substantially smaller than  $20^\circ$  although having acceptable performance become impractical to manufacture and use because of the overall depth of the burner plate (as will be apparent

from the further discussion below) and fragility of the peaks.

Another important characteristic of the combustion surface geometry is the spacing between apexes of adjacent peaked protrusions, which governs the depth of the valley portions between the peaked protrusions. This spacing between adjacent apexes should be at least  $\frac{1}{8}$  inch, and preferably between  $\frac{1}{4}$  to  $\frac{1}{2}$  inch. A spacing of  $\frac{1}{4}$  inch was used in burner plates from which the plotted data of FIGURE 7 was obtained.

The minimum spacing of  $\frac{1}{8}$  inch appears to be a limit at which significantly practical results are obtained, and below which improvements are too insubstantial to be noticeable. The spacing can be made as much as one inch or more but the distance between the peaks becomes so great that interparticle reinforcement is substantially decreased and performance reduced.

Ceramic honeycomb or perforated structures that are used for burner plates in accordance with the present invention should have certain particular characteristics that are necessary for proper operation without incurring detrimental flashback. First, the gas paths 25 should have a cross-sectional area at the combustion surface that does not exceed 0.006 square inch and a minimum length of about 0.2 inch, the latter being the minimum distance between surface 27 and the lowermost part in the valleys between peaked protrusions or surface 28. The gas passages, of course, should be substantially uniformly distributed throughout the burner plate and their cross-sectional areas in the aggregate should provide at least 20%, and more preferably at least 50%, of the total area of the combustion or radiating surface. When this total aggregate open area is 50% or more, the ceramic walls will necessarily be quite thin (i.e. 0.01 inch or less) and the upwardly flowing gas will extract most of the heat conducted down the wall of most any suitable ceramic material used, thereby preventing the well known undesirable effect of flashback from occurring. In the case where the total aggregate open area is less than 50%, with correspondingly thicker walls, the ceramic material used for the burner plate should desirably have a low heat conductivity on the order of less than 0.0020 cal./sec. cm.  $^{\circ}\text{C}$ . since the greater mass of the walls makes it less possible for the upwardly flowing gases to extract enough heat from higher heat conductivity ceramic walls to prevent flashback.

By way of illustration, and not of limitation, the following is given as the best mode contemplated of making burner plates according to this invention. A ceramic honeycomb body is prepared by coating a suitable carrier with a mixture of a pulverized ceramic and a binder, crimping the resulting coated carrier and then assembling it to the desired shape, alone or with another coated carrier that need not be crimped. The assembled body is then heated to a temperature sufficient to sinter it to a unitary structure as more fully detailed hereinafter. This procedure is, generally, the process set forth in the co-pending application of R. Z. Hollenbach, Serial Number 759,706, filed September 8, 1958, and now Patent No. 3,112,184, to which reference may be had.

The purpose of the binder is to bond the unfired ceramic material to the carrier, to impart green strength to the coated carrier and to retain the formed unfired article in the desired shape after forming and prior to sintering. It is preferred to use an organic binder that is curable or thermosetting and that can be removed by decomposition and/or volatilization when the honeycomb body is fired, such as epoxy resins.

The purpose of the carrier is to provide support for the unfired coating to allow it to be formed to the desired shape prior to sintering the ceramic coating. Tea bag paper is a preferred carrier because it will substantially decompose upon firing and thus result in an article consisting almost entirely of ceramic material.

Other suitable binders and carriers are disclosed in the

aforementioned Hollenbach patent application, to which reference can be made.

In order to produce a burner plate structure with optimum desirable characteristics of strength, low coefficient of thermal expansion (e.g.  $-10$  to  $+20 \times 10^{-7}/^{\circ}\text{C}$ .), thermal shock resistance and high specific heat, it is preferred to use lithium aluminosilicate ceramic materials such, for example, as glass or crystalline petalite and beta spodumene, glass-ceramics having a lithium aluminosilicate base (e.g. those made in accordance with Example 1 of United States Patent Number 2,920,971 to Stookey), as well as mixtures of any of the foregoing materials. Petalite glass-ceramic mixtures generally include about 10 to 40 weight percent of the glass-ceramic and the remainder petalite. Beta spodumene-petalite mixtures usually contain about 1 to 4 parts of petalite for each 4 to 1 parts of beta spodumene. These materials normally are used in a particle size of about minus 200 mesh (Tyler) or finer.

Structures are assembled from ceramic coated carriers in a variety of ways, and the resulting structures are called honeycombs, a term which in this specification means a unitary body having a multitude of unobstructed gas paths of predetermined size and shape, each such gas path being defined by thin ceramic walls and extending between and terminating in opposed major surfaces. These structures can be assembled from multiple layers of ceramic coated carriers corrugated with the same pattern with alternate layers laterally disposed a distance equal to half of the width of the individual pattern so that layers do not nest with each other. They can also be made from multiple layers of corrugated ceramic coated carriers with alternate layers having the corrugations angled in opposite directions from the perpendicular to the edge of the sheet. The honeycomb structure can also be formed from rolling up alternate layers of crimped and uncrimped coated carriers until the desired shape is formed. The structure can also be formed by assembling to a stack alternate crimped and uncrimped coated carriers until the desired dimensions are attained. The structure is made large enough to form the peaked protrusions on one major surface, as by cutting or sawing, and to provide a minimum gas flow path length of at least 0.2 inch. Other ways of making and assembling these honeycombs will be apparent to those skilled in the art.

The firing of the green structure or matrix, however formed, is accomplished in the normal manner for ceramic firing by placing the structure in a furnace and heating it at a rate slow enough to prevent breakage up to a temperature high enough to cause the ceramic particles to sinter. While the firing schedule, including heating rates and sintering temperatures, will vary depending upon the ceramic material utilized, the size and shape of the structure formed, and the atmosphere used, the details of such schedules are not critical and suitable conditions are readily determinable by one skilled in the art of firing ceramic article.

The invention will be described further in conjunction with the following example in which the details are given by way of illustration and not by way of limitation.

A ceramic composition was made of 75 parts by weight of petalite and 25 parts by weight of a glass-ceramic having the following approximate composition, by oxide analysis, in weight percent: 70%  $\text{SiO}_2$ , 18%  $\text{Al}_2\text{O}_3$ , 5%  $\text{TiO}_2$ , 3%  $\text{LiO}_2$ , 3%  $\text{MgO}$  and 1%  $\text{ZnO}$ . The composition was ball-milled to a minus 200 mesh (Tyler) particle size. A solution of the following composition was added to 2160 grams of the ceramic material in the ball mill:

|                          |
|--------------------------|
| 640 cc. of isopropanol   |
| 860 cc. of ethyl-acetate |
| 180 cc. of Versamid 115  |
| 480 cc. of Hysol 6111    |

75 Versamid 115 is the trade name of a thermoplastic poly-

mer supplied by General Mills, Inc. It is prepared by condensation of polymerized unsaturated fatty acids, such as dilinoleic acid, with aliphatic amines, such as ethylene diamine. Hysol 6111 is the trade name of an epoxy resin solution, supplied by Houghton Laboratories, Inc., containing 57% by weight of epoxy resin having a viscosity of about 2.5-4.0 poises at 25° C., and epoxide equivalent (grams of resin containing 1 g. chemical equivalent of epoxy) of 595±50, and a melting range of 73-85° C.

The ceramic material and the binder were further ball-milled for about three hours to produce a uniform suspension. A porous natural cellulose paper, commonly known as 3½ pound tea bag paper, cut to a width of 4 inches was then dipped into the suspension and dried by heating to 120° C. for 2 minutes. The dried, coated paper was then heated to 180° C. and crimped to produce a pattern, taken in cross-section, in the shape of a triangle with a height of about 0.04 inch and an open base of about 0.075 inch wide. The crimped, unfired, coated paper is rolled up simultaneously with a sheet of tea bag paper of the same width, which has been coated in the same manner but not crimped, upon a 2-inch diameter reel until an annular cylinder with an outside diameter of about 20 inches is obtained. Preferably, the uncrimped coated paper is not dried prior to the roll-up operation, but, as in the present example, this coated paper is dried by forcing air heated to about 120° C. through the channels of the annular cylinder as they are formed during the roll-up operation.

The unfired honeycomb body is then placed in a furnace chamber and heated in accordance with the following schedule:

| Temperature range     | Firing rate   |
|-----------------------|---------------|
| Room temp. to 700° C. | 350° C./hr.   |
| Hold at 700° C.       | 1 hour.       |
| 700° C. to 1220° C.   | Furnace rate. |
| Hold at 1220° C.      | 30 minutes.   |
| Cool to room temp.    | Furnace rate. |
| Refire to 1240° C.    | 300° C./hr.   |
| Hold at 1240° C.      | 7 hours.      |

Thereafter the honeycomb is cooled to handling temperature.

Burner plates were then sawed from the above honeycomb structure with a minimum gas flow path length of about ¾ inch and with square base pyramidal peaked protrusions having a ¼ inch spacing between adjacent apexes. Some were made with a 30° included angle between adjacent pyramidal surfaces and others with a 45°, 60°, 75°, 90°, 105° and 120° included angles. These burner plates were cemented to a ceramic burner body as shown in FIGURE 1.

Ceramic infrared gas burner plates prepared as just described were actually tested and found to be free from "dark" or cool zones on the radiating surface. The radiating surface temperatures were significantly higher (see FIGURE 7) and the heat radiation was more uniform than the previously made flat combustion surface ceramic burner plates. Moreover, significantly greater combustion of the gaseous fuel, i.e. natural gas and air, was also obtained as was evident by the considerable reduction of the CO content of the combusted gases being given off from the burner plate.

In accordance with the provisions of the patent statutes, I have explained the principle of my invention and have illustrated and described what I now believe to represent its best embodiment. However, it should be understood

that, although the present invention has been described with respect to specific details of certain embodiments thereof, it is not intended that such details be limitations upon the scope of the invention, except insofar as set forth in the appended claims.

What is claimed is:

1. A gas burner plate comprising a thin walled ceramic honeycomb having an inlet surface and an opposed combustion surface, a plurality of unobstructed gas passages uniformly distributed throughout the honeycomb and extending between and terminating in said surfaces, said passages being defined and separated from one another by thin walls of ceramic, each said passage having a cross-sectional area not exceeding 0.006 square inch, the aggregate cross-sectional areas of the gas passages providing an open space of at least 20% of the area of said combustion surface, at least a portion of said combustion surface having a configuration comprising a plurality of peaked protrusions, adjacent peaked protrusions having adjacent sloping surfaces forming an included angle therebetween of about 20 to 120° and having apexes spaced at least a distance of ½ inch whereby a plurality of said gas passages terminate in the sloping surfaces of each said peaked protrusion, and the length of all said gas passages being at least about 0.2 inch.

2. A gas burner plate according to claim 1 in which the peaked protrusions are pyramidal shape.

3. A gas burner plate according to claim 1 in which the peaked protrusions are conical shape.

4. A gas burner plate comprising a thin walled ceramic honeycomb having an inlet surface and an opposed combustion surface, a plurality of unobstructed gas passages uniformly distributed throughout the honeycomb and extending between and terminating in said surfaces, said passages being defined and separated from one another by thin walls of ceramic, each said passage having a cross-sectional area not exceeding 0.006 square inch, the aggregate cross-sectional areas of the gas passages providing an open space of at least 50% of the area of said combustion surface, said combustion surface having a configuration comprising a plurality of peaked protrusions, adjacent peaked protrusions housing adjacent sloping surfaces forming an included angle therebetween of about 30° to 90° and having apexes spaced a distance of about ¼ to ½ inch whereby a plurality of said gas passages terminate in the sloping surfaces of each said peaked protrusion, and the length of all said gas passages being at least about 0.2 inch.

5. A gas burner plate according to claim 4 in which the peaked protrusions are pyramidal shape.

6. A gas burner plate according to claim 4 in which the peaked protrusions are conical shape.

7. A gas burner plate according to claim 4 in which the ceramic honeycomb is formed of a lithium aluminosilicate material.

8. A gas burner plate according to claim 5 in which the ceramic honeycomb is formed of a lithium aluminosilicate material.

#### 60 References Cited in the file of this patent

#### UNITED STATES PATENTS

|                 |         |               |
|-----------------|---------|---------------|
| 1,731,053       | Lowe    | Oct. 8, 1929  |
| FOREIGN PATENTS |         |               |
| 65              | 551,940 | Belgium       |
|                 | 558,007 | Belgium       |
|                 | 626,559 | Canada        |
|                 |         | Nov. 14, 1956 |
|                 |         | June 29, 1957 |
|                 |         | Aug. 29, 1961 |

UNITED STATES PATENT OFFICE  
CERTIFICATE OF CORRECTION

Patent No. 3,170,504

February 23, 1965

John G. Lanning

It is hereby certified that error appears in the above numbered patent requiring correction and that the said Letters Patent should read as corrected below.

Column 3, line 53, for "aparent" read -- apparent --; column 5, line 12, for "obtained" read -- attained --; line 27, for "or" read -- on --; column 8, line 42, for "housing" read -- having --.

Signed and sealed this 24th day of August 1965.

(SEAL)

Attest:

ERNEST W. SWIDER  
Attesting Officer

EDWARD J. BRENNER  
Commissioner of Patents